

# UNITED STATES PATENT OFFICE.

WILLIAM AUGUSTUS HALL, OF NEW YORK, N. Y., ASSIGNOR TO AMERICAN MAHOGANY COMPANY, A CORPORATION OF MAINE.

## ART OF COLORING WOOD.

No. 901,095.

Specification of Letters Patent.

Patented Oct. 13, 1908.

Application filed June 29, 1906. Serial No. 324,027.

*To all whom it may concern:*

Be it known that I, WILLIAM AUGUSTUS HALL, a citizen of the United States, residing at New York, in the county of New York and State of New York, have invented or discovered certain new and useful Improvements in the Art of Coloring Wood, of which the following is a specification, reference being had therein to the accompanying drawings.

This invention has for its object to produce, from a comparatively inexpensive wood, a product closely resembling mahogany or other high-priced wood, both in its appearance and texture. This object is accomplished by a novel treatment of an inexpensive wood so as to give it the appearance and texture, throughout its body, of the more costly wood.

Attempts have heretofore been made to produce imitations of mahogany and other high priced woods, from less expensive hard woods, by forcing a staining dye or liquid into the comparatively cheap woods; but in order to secure satisfactory results, by the processes heretofore employed, it has been found necessary, in forcing the coloring solutions into the wood, to use exceedingly high pressures of from 800 to 1000 pounds to the square inch, or thereabout. Such high pressures have required very strong and costly tanks or cylinders of comparatively small diameters and capacities, so that the process of staining the wood has been so slow and costly that it has never gone into commercial use, to any considerable extent, so far as I am informed.

My invention has for its object to overcome the difficulties heretofore encountered by a process which will enable the use of comparatively small amounts of coloring matter, and which can be carried into effect by the use of tanks or pressure cylinders of much greater capacity and lower cost than those heretofore required; in that the wood is first softened and its fibers somewhat loosened or opened, and is also largely stained or darkened to a brownish red by a cooking process; is then rendered absorbent by a suction process which exhausts the liquor or water from the wood, and the wood is then further stained or darkened and its grain developed by forcing liquid coloring matter into the same; and this, owing to the absorbent condition of the wood, can be car-

ried into effect at comparatively low pressures and in tanks or receptacles much larger and less expensive than those heretofore required, where extremely high pressures for forcing the coloring or staining materials into the wood were necessary.

In carrying the invention into effect I take a hard wood (preferably yellow birch) in the form of deals, planks, boards or otherwise, and cook the same, by boiling in water in a closed tank or receptacle under a steam pressure of approximately 30 to 45 pounds pressure to the square inch, thus securing cooking temperatures of from about 250° to 275° F. This cooking operation is continued from one to three or four hours, according to the thickness of the wood, or until the resinous and gelatinous properties of the wood are thoroughly softened and the fiber of the wood somewhat loosened. This boiling or cooking, at the high temperatures referred to, also gives to the wood a reddish or brownish color which results from a stain due probably to a change in the ligno-cellulose compounds of the wood. The wood is then subjected to suction in a vacuum tank or chamber from which the air may be so far exhausted that the suction will draw the liquor or water out of the wood, so far as is practicable, so as to leave the wood in a more absorbent condition than it otherwise would be. After the wood has been thus rendered absorbent, and for the purpose of further coloring the same, a suitable liquid coloring matter, which will preferably contain salts of tannin and logwood or hemlock extract, is then put into the tank in which the wood is inclosed, and is forced into the pores of the wood preferably by a high hydraulic pressure; this operation being continued until the wood is impregnated with the coloring matter to such a degree that when the wood is dried it will closely resemble mahogany or other high priced wood, both in appearance and texture, according to the character of the staining material used for coloring or darkening the same. In this coloring process more of the coloring matter is absorbed in the lines of the grain cells or annular rings than in the other parts of the wood, so that the coloring matter is not uniformly deposited; and thus the "grain" of the wood is strongly brought out or intensified, thereby resulting in contrasting effects which enhance the beauty and value of the lumber. This result is

largely due to the fact that the vacuum treatment more thoroughly exhausts the moisture from the more porous parts of the wood occurring in the grain cells or annular rings, thereby rendering these parts more absorbent than the denser parts, so that they will take up more of the coloring matter, and thus the "grain" of the wood becomes very strongly developed, as just stated.

10 By first darkening or coloring the wood by the cooking process referred to a very great saving of the dye or coloring material is effected, as the wood will be partly colored by the cooking process and can then be colored 15 to the desired dark shades by a comparatively small amount of the stains or dyes.

So far as has been shown by the experiments which have been made in this matter, yellow birch is the most suitable hard wood 20 for being converted into imitation or artificial mahogany by the process above described, in that the grain or texture of this wood, after having been subjected to the described process, is almost identical with the 25 grain or texture of real mahogany. Other hard and comparatively inexpensive woods may, however, be subjected to the same treatment, without departing from the invention, and similar results be thereby 30 cured.

Having thus described my invention or discovery I claim and desire to secure by Letters Patent:

1. The herein described process of produc-

ing imitation of high-priced woods, consisting in cooking a comparatively inexpensive wood in water and at a temperature or temperatures exceeding 240° F. until the same is stained or darkened, then subjecting the wood to a vacuum process so as to suck the 40 water out of the wood so far as possible, and then further coloring or darkening the wood and developing the grain thereof by forcing a liquid coloring matter into the wood by pressure in a closed receptacle.

2. The herein-described process of producing imitation of high-priced woods, consisting in cooking a comparatively inexpensive wood in water and at a temperature or temperatures exceeding 240° F. until the gelatinous and resinous properties thereof are softened and the wood is darkened throughout, then subjecting the wood to a vacuum process for the purpose of sucking the liquid out of the wood so far as possible, and finally 55 impregnating the wood, thus rendered absorbent by the vacuum process, with a liquid coloring matter which is forced into the wood under pressure so that the coloring matter becomes largely deposited in the annular 60 rings and grain cells, thereby intensifying or developing the "grain" of the wood.

- In testimony whereof I affix my signature, in presence of two witnesses.

WILLIAM AUGUSTUS HALL.

Witnesses:

HENRY CALVER,  
C. M. SWEENEY.